

## UNITED STATES PATENT OFFICE.

JOHN H. WHITE, OF CRANFORD, NEW JERSEY, ASSIGNOR TO WESTERN ELECTRIC COMPANY, INCORPORATED, OF NEW YORK, N. Y., A CORPORATION OF NEW YORK.

## CASTING METALS.

No Drawing. Continuation of application Serial No. 683,320, filed December 29, 1923. This application filed December 29, 1924. Serial No. 758,584.

This invention relates to casting of metals and metal alloys.

It is the general practice in the casting of metals and metal alloys to place the mass to be melted in a crucible or other receptacle, raise the temperature to the melting point of the metal, or to the highest melting point of the constituent elements of an alloy, and to pour the molten metal into a mold. 10 If the cast metal is to be worked instead of being left in the form in which it is cast, the mold is usually of such shape as to produce a rod-like or plate-like ingot. At the open end or side of the mold into which the molten metal is poured, there is formed a depression as the metal solidifies. This depression, in the case of a rod-shaped ingot, is called a pipe and may extend a third of the length of the rod, necessitating the discarding of a 15 third of the ingot at the top. If the entire ingot is rolled or otherwise worked, a seam develops from the pipe. It is customary to add molten metal as this depression forms for the purpose of filling it, but at best this 20 portion of the ingot is of a different character than the rest, and may result in the development of flaws or faults during subsequent working. The formation of the pipe is due, it is generally agreed, to the forcing 25 out of gas from the molten mass at the instant of solidifying.

As an expedient sometimes adopted for preventing the formation of a pipe or other depression for example in the casting of iron, the molten metal is caused to drop rapidly in temperature so that the dissolved 30 gases are entrapped when solidification occurs and, instead of separating entirely at one end of the ingot and forming a pipe, are disseminated throughout the mass of metal in the form of large or small blow holes. During subsequent working the blow holes are closed and a perfect welding of the metal takes place. But, as explained below, 35 it has been found that welding does not occur with all metals and metal alloys, and probably perfect welding in the case of alloys is the exception rather than the rule. A method which is sometimes used where it is desired to avoid blow holes is to raise the temperature of the molten metal, add a degasifying agent and then reduce the temperature very slowly to permit the gases to escape completely. But this method does

not do away with the formation of the depression mentioned above. 45

When a pipe is formed, if impurities are present, the walls of the pipe are likely to be of metal of different character than the deeper portion of the casting. This appears 50 to be due to the uniting of the impurities with the principal metal or metals to form alloys or compounds having lower melting points than the principal metal or alloy, in which case they are segregated around the 55 pipe. For example, if sulphur and phosphorous are present in iron as impurities, a casting will have layers of iron phosphides and sulphides adjacent the pipe.

A further difficulty experienced with alloy 60 ingots formed by processes now in general use is that they are likely to tear apart in the mold during cooling due to their lack of toughness.

It has heretofore been proposed to improve 65 the quality of metal ingots by melting the metal or alloy in a gas-tight electric furnace under subatmospheric pressure, exhausting the furnace to produce as high a vacuum 70 therein as may be necessary for the metal to 75 be treated, during the whole process maintaining the furnace at a substantially constant temperature depending upon the metal or alloy being treated, and exhausting the 80 gases therefrom until, with the furnace hermetically closed, no increase of pressure 85 therein is observed even after the metal or alloy has solidified; the metal being then cooled and removed from the furnace, remelted and cast in the usual manner. This 90 process overcomes many of the defects noted above, but is very expensive.

It is the principal object of this invention to overcome some or all of the above 95 noted defects in metal castings in a simple and cheap manner and to produce castings which are free from pipes and blow holes, are sound, tough and nearly or quite homogeneous in structure.

The invention is based upon the discovery 100 that if the molten metal is melted in the presence of air at atmospheric pressure and is permitted to cool until it solidifies and then is very soon reheated and poured, the resulting casting will be of the improved 105 character just stated. If the metal after solidifying and before remelting is permitted to stand for some time or to cool to

room temperature, many or all of the above noted defects will be present in the casting.

The reason for the improved result is not known, but it is thought that it may be due

5 to an expulsion of occluded gas into the metal during the first solidifying, which forms gas pockets, the gas in which, however, is unable to escape, because almost coincident with the expulsion of the occluded gas

10 the mass of metal becomes rigid and entraps it, and the subsequent melting permits the entrapped gas to escape. It is immaterial, however, what is the correct theory, since, to practice the invention it is only necessary to

15 know the results obtained and the process used in obtaining them. No noticeable additional benefit is derived from continuing this process of remelting beyond this first stage. It seems probable that the ill effect of per-

20 mitting the metal to stand even for a short time after solidifying and before being remelted, is due to a rapid absorption of air or gases. To obtain the best results, therefore, the remelting must be done immediately

25 after solidification has occurred. Likewise, to obtain the best results, pouring should take place immediately after reheating, as otherwise gas is apparently absorbed by the molten metal.

30 The invention is the outgrowth of an extended research to discover the best method of making nickel-iron alloy wire and tape, the preferred proportions of the alloy being about 80% of nickel and 20% of iron. When

35 ingots were cast in accordance with usual methods, the results were very unsatisfactory. A deep pipe formed in the ingot necessitating much waste. When the ingots were rolled there developed transverse cracks

40 which did not weld during further working. Frequently the ingot was torn apart in the mold during cooling. The casting was not homogeneous or tough and had to be annealed before it could be worked.

45 In the practice of the invention the preferred procedure in the case, for example, of a nickel-iron alloy, is as follows: The iron and nickel are placed in the crucible or other receptacle in the desired proportions

50 and melted in the usual manner. The mass is then allowed to cool until it has solidified, after which it is again immediately melted and poured into the mold preferably immediately after this second melting. The

55 induction furnace is particularly well adapted for this process since it permits the reheating to be done at once after the solidification point has been reached. It is only necessary to stop the flow of current at the proper time and, after the required interval, to start it again.

60 This process has several marked advantages over that mentioned above in which the melting is done in a gas-light furnace and pumping is carried

on while the heat for melting is applied and subsequently thereto, a very high degree of vacuum being maintained. These advantages are (1) the cost of the equipment for carrying out the process is very much less; 70 vacuum furnaces require expensive auxiliary pumping apparatus and are not suitable for the final melting before casting; (2) the time required is very greatly reduced, not only because of the shorter time necessary before 75 the charge is permitted to solidify, but also because it is not necessary to wait for the charge to cool before remelting. If a vacuum furnace is employed, the charge must be removed from the furnace and re-heated in another so that the molten metal 80 can be poured.

85 This invention will find its principal application in the manufacture of alloys which are designed to have some particular quality or characteristic to a marked degree, such as permeability, toughness, hardness, etc. So-called special steels are in this class.

90 Steels which are now used as automobile parts, for example, are often "flakey" in structure, and this is thought to be due, in the light of the discoveries leading up to this invention, to the minute blow holes or entrapped gas in the casting, the walls of

95 which holes do not weld together perfectly during subsequent working of the metal, as would be the case if the casting were of iron alone. Larger faults in automobile parts

100 may result from the lack of homogeneity in the casting, from larger blow holes, and from incipient cracks introduced by rolling. When nickel-iron castings eight inches by three inches by one inch having about 80%

105 of nickel and 20% of iron were cast in accordance with this invention and compared with others made in the usual manner, it was found that the former could be rolled to thin sheets without being first annealed,

110 while the latter cracked after a few passes in the rolls, necessitating the discarding of all but a small portion of the sheets. The castings made by the improved process were sound and tough.

115 In the preparation of special steels, so called, and other alloys of the kind mentioned above, induction furnaces are ordinarily employed, since other furnaces are likely to introduce impurities into the melt. This invention can therefore be practiced

120 easily and cheaply in the manufacture of all such alloys. It is also applicable of course, though not quite so readily, to other furnaces. While the greatest use of the invention

125 is in connection with the manufacture of alloys or articles made from alloys, it is not limited to such use, as castings of pure metal, or metals of the degree of purity used for ordinary commercial purposes, when made according to this invention are of 130 superior quality.

This application is a continuation of an application of J. H. White, Serial No. 683-320, filed December 29, 1923.

What is claimed is:

- 5 1. The method of working a metallic composition containing large amounts of nickel which comprises melting together the component elements, cooling the melt until it solidifies, immediately remelting, casting 20 immediately after the remelting, and working the casting without first subjecting it to an annealing temperature.
- 10 2. The method of producing and working an alloy consisting chiefly of nickel and iron which comprises the steps of melting together the component elements, cooling the melt until it solidifies, immediately remelting, at once casting, and working the casting without first subjecting it to an annealing temperature.
- 15 3. The method of producing and work-

ing a nickel-iron alloy consisting chiefly of nickel and iron in which the nickel component greatly exceeds the iron component, which method comprises the steps of melting together the component elements, cooling the melt until it solidifies, immediately remelting and at once casting, said steps being carried out without the use of a vacuum, and cold working the casting.

4. The method of producing and working an alloy consisting chiefly of nickel and iron, which comprises the steps of melting together the component elements, cooling the melt until it solidifies, immediately remelting, and at once casting, said steps being carried out without the use of a vacuum, and cold working the casting.

In witness whereof, I hereunto subscribe my name this 26th day of December A. D., 1924.

JOHN H. WHITE.